

July 22, 1952

A. W. HERBENAR

2,604,419

METHOD OF HEAT-TREATING SURFACE HARDENED ARTICLES

Filed April 7, 1949



FIG. 1



FIG. 3



FIG. 2



FIG. 4  
INVENTOR.

ANTON W. HERBENAR

BY

*Alfred C. Boddy*

ATTORNEY

## UNITED STATES PATENT OFFICE

2,604,419

METHOD OF HEAT-TREATING SURFACE  
HARDEDEN ARTICLESAnton W. Herbenar, Ferndale, Mich., assignor to  
The Ohio Crankshaft Company, Cleveland,  
Ohio, a corporation of Ohio

Application April 7, 1949, Serial No. 86,078

3 Claims. (Cl. 148—21.5)

1

This invention pertains to the art of metal heating and, more particularly, to the heating of metals for the purposes of drawing or tempering hardened layers or surfaces thereon.

An object of the present invention is to provide a new and improved method for drawing or tempering hardened layers or surfaces on metallic articles of manufacture which permits of ready control of the amount of draw, which permits of a substantially uniform draw throughout the entire hardened layer and which avoids the objections of the prior art.

Another object of the invention is to provide a new and improved method for drawing a hardened surface or layer on a metallic article of manufacture including the step of introducing, subsequent to the hardening operation, the heat for the drawing into the article on a side remote from the hardened surface.

Another object is the provision of a new and improved method of drawing a hardened surface on a curved or flat metallic member having adjacent surfaces in the relatively unhardened state which comprises applying heat, subsequent to the hardening operation, as by electric induction heating to the unhardened surface and allowing the heat to flow by conduction to the hardened surface.

The invention is applicable to any metallic article having a surface portion or layer which must be heated throughout its thickness uniformly and to a readily controlled amount.

The invention will be described as embodied in and applied to a cylinder liner which has an inner quench-hardened layer or surface, although it is equally applicable to other shapes of metallic articles either regular or irregular in shape or having continuous or discontinuous hardened surfaces.

Referring now to the drawings which are for the purposes of illustration only and not for limitation of the scope of the invention:

Figure 1 is a side sectional view of a portion of a cylinder liner having an inner hardened surface to be drawn to a lower hardness and an electric induction-heating head adjacent the hardened surface to supply the necessary heat;

Figure 2 is a graph showing a group of typical curves of wall hardness plotted against cylinder wall thickness and showing the hardness variations resulting from the method of heating shown in Figure 1;

Figure 3 is a view similar to Figure 1 but with the inductor for supplying the drawing heat positioned adjacent a surface of the liner remote

2

from the hardened surface and embodying the present invention; and

Figure 4 is a view similar to Figure 2 but showing typical hardness curves obtainable by the present invention.

Referring now to Figure 1, a portion of a cylinder liner 10 is shown formed of a material such as steel or the like having the characteristics which, in its initial unheat-treated state, is relatively soft throughout but which can be hardened by heating above a critical temperature and rapidly quenched. The liner 10 has an inner hardened layer or surface 11 integral with and immediately adjacent to an outer layer or surface 12 which is relatively unaffected by the heat-treating operation and, therefore, still relatively soft.

The hardened surface 11 can be produced by any conventional means but preferably by positioning an electric induction-heating head 13 interiorly of the liner and adjacent to the inner surface, thus inducing high-frequency electric currents to flow in the surface 11 to raise its temperature above the critical quench-hardening temperature. Subsequently, the surface is rapidly and forcefully quenched by a quench head or the like not shown.

Curve A of Figure 2 shows a typical hardness curve obtainable by using the above described electric induction heating and quench method. As shown by this curve, the initial hardness of the metal of the cylinder wall was 10 Rockwell C. The quench-hardening operation increased the hardness on the inner surface of the liner to 60 Rockwell C, which high hardness extended from the inner surface of the liner outwardly for about a third of the thickness of the wall and then dropped rapidly in a very short wall thickness to the initial hardness of 10 Rockwell C.

Such heat-treating methods oftentimes produce surfaces harder than are desired or produce surfaces which have high internal stresses therein which must be removed even at the sacrifice of some of the hardness of the surface. It is known that as the hardened surface or layer 11 is reheated to some temperature below the critical temperature, a softening of the hardened layer will result dependent on the temperature and the length of time that the layer is held at that temperature together with a simultaneous, very substantial relief of the internal stresses. This operation is called a drawing or tempering operation.

To perform this drawing operation on cylinder liners for example, it has been conventional

in the past to pass a high-frequency electric induction-heating head interiorly of the cylinder liner, heating the liner to the desired degree below the critical temperature and allowing it to cool. A heating head identical to the one used for the hardening operation may be employed by using a lower concentration of electrical energy; or, if progressive heating is used, by moving it faster. It has been found in practice that such a method of supplying the heat for drawing oftentimes produces an undesirable final hardness pattern in that the absolute outer surface of the hardened layer draws to a greater degree than the portions of the hardened layer more remote from the outer surface.

As an illustration of this fact, assume for example it is desired to draw the surface of the hardened layer to 44 Rockwell C. Curve B of Figure 2 is typical of the hardness pattern which will result. The surface area as shown by the curve will be of the required hardness. However portions intermediate the surface of the hardened layer and the unhardened portion 12 will be drawn to a lesser degree and will have a hardness somewhat between the desired 44 Rockwell C and the initial hardness.

Assume further that it is desired to obtain a maximum hardness of 44 Rockwell C through the hardened layer 11. Obviously, the temperature of the hardened layer must be increased or the layer must be held at this temperature for a longer period of time. Curve C of Figure 2 represents typical results. While the maximum hardness has been reduced to 44 Rockwell C, the hardness at the surface of the hardened layer 11 is substantially below that and is shown at 22 Rockwell C.

Without limitation on the scope of the invention but rather to aid in an explanation thereof, applicant advances the following theory for this variation in hardness pattern. As is known, high-frequency induced currents of the metallic article are concentrated almost entirely at and immediately below the surface of the member adjacent the induction-heating head. For producing hardened layers of shallow depth, this is extremely desirable but for drawing purposes, applicant advances the theory that this concentration of currents at the surface causes the variation in hardness pattern. As the entire cylinder wall is to be heated through, it is obvious from an examination of heat-flow theory that the source of the heat must be at some temperature above the portions of the wall to which the heat can flow by conduction. In the present instance, the source of the heat is interiorly of the metal itself but still adjacent a surface opposite the heating head. A temperature pattern somewhat as indicated by the curve  $t_1$  is believed to occur, the elevated portions of the curve being that where the currents themselves flow. It is believed that this accounts for the increased draw adjacent the inner surfaces of the cylinder liner.

The present invention contemplates a method of drawing metal articles having a hardened layer such as the cylinder of Figure 1 whereby an even temperature and thus drawing of the hardened layer 11 may be obtained throughout its entire thickness. Generally speaking, the invention comprises generating the drawing heat or introducing the drawing heat into the metal at a point remote from the hardened layer itself and allowing the heat to flow thereto by conduction. Further, generally speaking, the in-

vention comprises introducing the heat into areas of the metal where overheating has no ill effects and allowing this heat to flow by conduction into the hardened area.

Thus, in the embodiment of the invention shown, the cylinder liner 10 of Figure 1 with its internally hardened layer 11 has the heat applied externally thereto; that is, on the side remote from the hardened layer 11 and the heat is allowed to flow into the hardened layer by conduction. This process is in contra-distinction to that shown in Figure 1 where the heat is generated in the hardened layer itself. In the embodiment shown in Figure 3, an induction-heating coil 15 is positioned exteriorly of the cylinder liner 10 and is connected to a suitable source of high-frequency electric energy not shown. High-frequency heating currents still flow only adjacent the surface of the liner opposite from the induction-heating coil itself. No heating currents in the embodiment shown in Figure 3 will flow within the hardened layer. Thus, the heat is generated only in the soft portion 12 and flows to the hardened layer 11 by thermal conduction.

A temperature curve such as that indicated by  $t_2$  will generally exist across the thickness of the liner wall. It will be obvious from this curve that the temperature in the hardened layer itself will be substantially uniform throughout its entire thickness, that the higher temperatures generated in the wall are actually generated in the layer 12, which is essentially soft and will not be effected by heating to a temperature below the critical.

It is possible to obtain a more rapid heating by heating externally. For example, a higher rate of power can be applied initially resulting in the outer wall of the liner being at a more elevated temperature; for example, such as that shown by curve  $t_3$ . The flow of heat by conduction soon levels out the temperature.

It will be appreciated that the induction-heating coil 15 may be of any known type and may be progressively moved along the cylinder liner or may be held stationary.

Curve D of Figure 4 shows a typical hardness pattern resulting from the drawing operations following the teachings of this invention. It will be noted that this curve shows a substantially uniform hardness obtained through the hardened layer 11 after the drawing operation.

It will be obvious that the present invention is not limited to cylinder liners. It can be used on any other metallic articles having hardened or other layers produced by any known means. The hardened layers need not be electrically conductive. It is sufficient that the heating be generated elsewhere than in the hardened surface itself. Radiant heat in the embodiment shown in Figure 3 could be substituted for the induction-heating coil 15.

Other modifications will occur to others upon a reading and understanding of this specification. It is my intention to cover all such modifications insofar as they come within the scope of the appended claims.

Having thus described my invention, I claim:

1. The method of heat treating a metallic article of manufacture for the purpose of drawing a previously hardened surface layer portion thereof, said article having a body portion and a surface layer portion on each side of said body portion, one of said surface layer portions being previously hardened, which comprises subsequently applying heat to said other surface layer

portion to raise the temperature thereof above the temperature of said other portions of said article to conduct said heat through said body portion and into said previously hardened surface layer portion to draw said last portion.

2. The method of heat treating a cylindrical metallic article of manufacture for the purpose of drawing a previously hardened surface layer portion, said article having an outer cylindrical surface layer portion, an inner cylindrical surface layer portion and a body portion intermediate said surface layer portions, one of said surface layer portions being previously hardened, which comprises subsequently applying heat to said other surface layer portion to raise the temperature thereof above the temperature of said other portions of said article to conduct said heat through said body portion and into said previously hardened surface layer portion to draw said last portion.

3. The method of heat treating a metallic article of manufacture, said article having a body portion and a surface layer portion on each side of said body portion, which comprises heating

one of said surface layer portions to quench-hardening temperature, quench-hardening said surface layer portion, subsequently applying heat to said other surface layer portion to raise the temperature thereof above the temperature of said other portions of said article to conduct said heat through said body portion and into said quench-hardened surface layer portion to draw said quench-hardened surface layer portion.

10

15

20

ANTON W. HERBENAR.

## REFERENCES CITED.

The following references are of record in the file of this patent:

## UNITED STATES PATENTS

| Number    | Name    | Date          |
|-----------|---------|---------------|
| 2,295,272 | Somer   | Sept. 8, 1942 |
| 2,303,467 | Inskeep | Dec. 1, 1942  |

## FOREIGN PATENTS

| Number  | Country       | Date         |
|---------|---------------|--------------|
| 485,733 | Great Britain | May 19, 1938 |